# EUROPEAN PATENT SPECIFICATION

(11) **EP 1 504 831 B1**
(45) Date of publication and mention of the grant of the patent: **01.04.2009**
(21) Application number: 03721000.2
(22) Date of filing: 30.04.2003
(51) Int. Cl.: B22D 41/50, C04B 35/03, B22D 41/54

(54) **METHOD FOR CONTINUOUS CASTING OF ALUMINUM KILLED STEEL**
STRANGGIESSENVERFAHREN VON ALUMINIUMBERUHIGTEM STAHL
PROCEDE DE MOULAGE PAR COULEE CONTINUE D'UN ACIER CALME A L'ALUMINIUM

(30) Priority: 30.04.2002 JP 2002128337
(43) Date of publication of application: 09.02.2005
(73) Proprietor: Krosakiharima Corporation, Kitakyushu-shi, Fukuoka 806-8586 (JP); LWB Refractories Company, York, PA 17405-1189 (US)
(72) Inventor: Ogata, Koji, KROSAKIHARIMA CORPORATION, Kitakyushu-shi, Fukuoka 806-8586 (JP); Shimizu, Koichi, KROSAKIHARIMA CORPORATION, Kitakyushu-shi, Fukuoka 806-8586 (JP); Asano, Keisuke, KROSAKIHARIMA CORPORATION, Kitakyushu-shi, Fukuoka 806-8586 (JP); Hokii, Toshiyuki, KROSAKIHARIMA CORPORATION, Kitakyushu-shi, Fukuoka 806-8586 (JP); Yoshitomi, Joki, KROSAKIHARIMA CORPORATION, Kitakyushu-shi, Fukuoka 806-8586 (JP)
(74) Representative: Goddar, Heinz J.
(86) International application number: PCT/JP2003/005558
(87) International publication number: WO 2003/092929

(56) References cited:
- JP-A- 5 154 627
- JP-A- 5 285 612
- JP-A- 8 039 214
- JP-A- 2003 040 672
- PATENT ABSTRACTS OF JAPAN vol. 016, no. 331 (M-1282), 20 July 1992 (1992-07-20) & JP 04 094851 A (AKECHI SERAMITSUKUSU KK), 26 March 1992 (1992-03-26)
- PATENT ABSTRACTS OF JAPAN vol. 016, no. 452 (M-1313), 21 September 1992 (1992-09-21) & JP 04 158963 A (NIPPON STEEL CORP; others: 01), 2 June 1992 (1992-06-02)
- PATENT ABSTRACTS OF JAPAN vol. 017, no. 321 (C-1072), 18 June 1993 (1993-06-18) & JP 05 032456 A (TOKYO YOGYO CO LTD), 9 February 1993 (1993-02-09)
- PATENT ABSTRACTS OF JAPAN vol. 1996, no. 06, 28 June 1996 (1996-06-28) & JP 08 039214 A (KUROSAKI REFRACT CO LTD; others: 01), 13 February 1996 (1996-02-13)
- PATENT ABSTRACTS OF JAPAN vol. 017, no. 548 (M-1490), 4 October 1993 (1993-10-04) & JP 05 154627 A (SHINAGAWA REFRACT CO LTD), 22 June 1993 (1993-06-22)
- PATENT ABSTRACTS OF JAPAN vol. 018, no. 062 (M-1553), 2 February 1994 (1994-02-02) & JP 05 285612 A (KUROSAKI REFRACT CO LTD; others: 01), 2 November 1993 (1993-11-02)

## Description

### TECHNICAL FIELD

The present invention relates to a method of continuous casting of aluminum-killed steel using a continuous casting nozzle.

### BACKGROUND ART

In a process for casting of aluminum-killed steel, alumina inclusions are attached to the surface of an inner hole of a nozzle unit for use in casting (hereinafter referred to as "nozzle unit" for brevity), and agglomerated to form a large-size alumina particles. The agglomerated alumina particles are mixed in the molten steel flow, and incorporated into slabs as large-size inclusions to cause defect or deteriorated quality in the slabs.

In particular, as to aluminum-killed steel which is molded as high-grade steel, such as thin sheets, it has been recently required to strictly control the quality of steel products. To meet this requirement, a good deal of effort has been made to prevent alumina from being attached onto the surface of an inner hole of a nozzle unit for use in pouring molten steel from a tundish (hereinafter referred to as "TD") into a mold in a continuous casting process.

As one of measures against the attachment of alumina, there has been known a method comprising injecting argon gas from the inner surface of a nozzle unit into molten steel to physically prevent the attachment of alumina. In this method, if the argon gas is injected at an excessive amount, bubbles of the injected argon gas will be incorporated into molten steel to form pinholes in slabs or cause defect thereof. Thus, due to the restriction in the allowable injection amount of argon gas, this method cannot be exactly used as a sufficient measure for preventing the attachment of alumina.

As another measure, there has also been known a method intended to provide a function of preventing the attachment of alumina, to a refractory material itself constituting a nozzle unit. This method is directed to prepare a refractory brick containing CaO and induce the reaction between the CaO and alumina attached onto the brick to form a low-melting-point compound so as to prevent the attachment of alumina from further increasing. For example, Japanese Patent Publication No. 61-44836 discloses a casting nozzle unit using refractories which comprise a primary component consisting of a combination of graphite, and sintered or fused calcia or another ceramic engineering material containing a CaO component.

Generally, a nozzle unit for use in pouring molten steel from a TD to a mold during casting of steel includes a multi-part type nozzle unit constructed by combining a plurality of segmental nozzles as shown in FIG. 1, and a single-part type nozzle unit consisting of only a single-piece nozzle as shown in FIG. 2.

The multi-part type nozzle unit is constructed by combining an upper nozzle 2 which is attached to an opening formed in the bottom wall of a tundish 1, a sliding nozzle 3, a lower nozzle 4, and a submerged or immersion nozzle 5 immersed in a mold 6. The flow rate of molten steel to the mold 6 is controlled by adjusting the opening area of the sliding nozzle 3. The multi-part type nozzle unit has an excellent flow-rate control function, and can stably maintain the level of molten steel. Thus, the multi-part type nozzle unit is widely used in view of stable casting performance under constant conditions and excellent safety.

The single-part type nozzle unit is comprised of a single elongated immersion nozzle defining a flow path which extends from the bottom opening of the tundish 1 to the mold 6. The flow rate of molten steel to the mold 6 is controlled by adjusting the area of the bottom opening of the tundish 1 using a long stopper 7 disposed in the tundish 1.

In experimental tests using the above two types of nozzle units each of which has an inner hole whose surface is formed of the aforementioned material containing CaO, the single-part type nozzle unit as shown in FIG. 2 actually exhibited an effect of reducing the attachment of alumina to the inner hole surface thereof and reducing large-side alumina inclusions. On the other hand, it was proven that when the CaO-containing material is applied to only a part of the segmental nozzles of the multi-part type nozzle unit as shown in FIG. 1, large-size alumina inclusions in slabs tend to be formed at a larger amount that that in the single-part type nozzle unit.

In a casting process using the single-part type nozzle unit, molten steel passing through the nozzle unit has substantially no contact with outside air. By contrast, in a casting process using the multi-part type nozzle unit, outside air enters in the inner hole through joints between the segmental nozzles. In particular, outside air inevitably inflows through the joint surface between the sliding nozzle (hereinafter referred to as "SN") and the associated segmental nozzle, because it is difficult to completely seal the joint surface with the SN to be slidingly moved during use.

The molten steel for aluminum-killed steel contains aluminum dissolved therein. When the aluminum comes into contact with air, it is oxidized to create alumina. Then, the created alumina becomes incorporated into slabs as alumina inclusions. In the multi-part type nozzle unit composed of the plurality of segmental nozzles, even if the CaO-containing refractories are applied to a part of segmental nozzles, alumina will be attached to the remaining segmental nozzles having no CaO-containing refractories, and then large-sized alumina due to agglomeration will be incorporated into slabs.

JP-A-494851 (abstract) discloses a nozzle for continuous casting for stably restraining harrowing and further clogging of an inner hole caused by non-metallic inclusion. The inner hole in the nozzle for pouring the molten steel consists of 50-89wt.% of calcium zirconate containing CaO ZrO₂ as the essential component as mineral composition, 10-35% graphite and 0.5-10% fluoride containing calcium fluoride.

JP-A-5154627 (abstract) discloses a refractory composition for preventing stickness and deposition of non-metallic inclusions. In the inner hole surface layer contacting with the molten steel in an immersion nozzle composed of alumina-graphite composition, another composition is arranged. This composition is constituted of 65-80wt.% of zirconia clinker containing calcia, magnesia and silica, graphite and silicon carbide.

JP-A-5032456 (abstract) discloses a refractory material which is composed essentially of CaO, SiO₂ and B₂O₃ wherein the sum of CaO, SiO₂ and B₂O₃ in the total refractory is ≤ 95wt.%.

JP-A-8039214 (abstract) discloses a nozzle for continuous casting which is made of an alumina-graphite refractory, and a zirconia-graphite refractory is fitted to a slag line and a refractory layer without containing the carbon is arranged on the inner hole surface and the outer periphery at the lower part thereof through a joint filler.

JP-A-4158963 (abstract) discloses a nozzle for continuous casting, the neighborhood of the inner hole in the nozzle is made to two or more layers of multi-layers structure. The inner hole surface side is formed with a high CaO component layer composed of 15-30wt.% CaO 40-80% ZrO₂ 5-40% graphite and less than 10% of other refractory components.

JP-A-5285612 (abstract) discloses a nozzle inner hole body for continuous casting. The inner hole body is composed of mixed powder of powder of 2-40wt.% in conversion into CaO and one or more alumina clinker, spinel clinker and magnesia clinker.

### DISCLOSURE OF INVENTION

It is an object of the present invention to provide a method for continuous casting of aluminum-killed steel using a continuous casting nozzle, capable of significantly reducing the amount of large-size alumina inclusions in slabs to achieve a reduced quality-defect rate.

This object is achieved by the method of claim 1. Preferred embodiments are disclosed in the subclaims.

Through various research on the amount of large-size aluminum inclusions in slabs obtained using a single-part type or multi-part type nozzle unit which has an inner hole to be used for pouring molten steel from a tundish to a mold therethrough and CaO-containing refractories applied to a surface of the inner hole, it was found that the amount of large-size aluminum inclusions in slabs has a strong correlation with the entire surface area of the inner hole of the nozzle unit and the amount of CaO contained in the employed refractories. Based on this knowledge and obtained specific numerical requirements, the present invention has been accomplished.

Specifically, according to the present invention, more than 50 % of the entire surface area of an inner hole of a nozzle unit to be used for pouring molten steel from a tundish to a mold is formed of refractories containing 20-60 mass% of CaO.

In the multi-part type nozzle unit as shown in FIG. 1, even if CaO-containing refractories are applied to a part of the segmental nozzles or to define a portion of the entire surface area of the inner hole, alumina will be attached onto the inner hole surface of the remaining segmental nozzles having no CaO-containing refractories, and large-sized alumina due to agglomeration will be undesirably incorporated into slabs.

When the refractories containing 20 mass% or more of CaO are applied to the inner hole of the nozzle unit for allowing molten steel to flow down therethrough, in such a manner that the CaO-containing refractories occupy 50 % or more of the entire surface area of the inner hole, the amount of large-size alumina inclusions in obtained slabs is drastically reduced. This effect is derived from a synergistic effect of the actions, of which the CaO-containing refractories act to absorb alumina, a low-melting-point compound created through the reaction between CaO and alumina in the form of a liquid phase acts to smooth the inner hole surface, as well as prevention of the attachment of alumina and prevention of the agglomeration of alumina.

Such a synergistic effect can be obtained only if the CaO-containing refractories are applied to the surface of the inner hole of the nozzle unit, in such a manner that they occupy more than 50 % of the entire surface area of the inner hole. If the ratio is less than 50 %, the action of reducing the amount of alumina flowing into the mold is deteriorated to provide only an insufficient effect of reducing the amount of large-size alumina inclusions in the slabs. The ratio should preferably be set at 60 % or more. While 100 % of the entire surface area of the inner hole of the nozzle unit may be formed of the CaO-containing refractories, the CaO-containing refractories should be selectively applied to an appropriate region of the nozzle unit in consideration of its use conditions. For example, if a certain region has the risk of causing a problem, such as fusion damage or abrasion, in conjunction with the use of the CaO-containing refractories, suitable conventional refractories for such a region should be used.

The present invention can be applied to any multi-part type nozzle unit composed of either one of a combination of an upper nozzle and an immersion nozzle, a combination of a SN and an immersion nozzle, a combination of an upper nozzle, a SN and an immersion nozzle, and a combination of an upper nozzle, a SN, an lower nozzle and an immersion nozzle as shown in FIG. 1, and to any single-part type nozzle unit composed of a single-piece immersion nozzle as shown in FIG. 2, in such a manner that the CaO-containing refractories occupy more than 50 % of the entire surface area of the inner hole of the nozzle unit. Further, the present invention can also be applied to a multi-part type nozzle unit in which a SN is integrated with an upper or lower nozzle in a single piece. Even in case where the CaO-containing refractories are applied to only a portion of the surface of the inner hole of the single-part type nozzle unit, if they are applied to occupy or define more than 50 % of the entire surface area of the inner hole of the nozzle unit, the quality of slabs can be significantly improved.

If the amount of CaO to be contained in the refractories for defining a surface of the inner hole is less than 20 mass%, the refractories have deteriorated abilities of absorbing alumina and preventing the attachment of alumina to provide only an insufficient effect of reducing the amount of large-size alumina inclusions in slabs. Thus, the amount of CaO must be 20 mass% or more.

While there is no upper limit of the amount of CaO to be contained in the refractories in terms of the effect of reducing the amount of large-size inclusions in slabs, a large amount of CaO is likely to cause the increased risk of fusion damage or wearing. Thus, the upper limit of the amount of CaO should be appropriately adjusted depending on its use conditions. In usual casting conditions, the amount of CaO is set at about 60 mass% to obtain sufficient effects.

The refractories include MgO-CaO-C based refractories.

In the single-part type or multi-part type nozzle unit, the CaO-containing refractories are essentially applied to at least a surface of the inner hole to be in contact with molten steel. Any region of the nozzle unit other than the inner hole surface may be made of the same material as that of the inner hole surface, or may be made of any suitable refractories used in a conventional nozzle unit.

### BRIEF DESCRIPTION OF DRAWINGS

FIG. 1 is a schematic sectional view showing a multi-part type nozzle unit composed of a plurality of segmental nozzles including a SN, which is one example of a nozzle unit to which the present invention is applicable.
FIG. 2 is a schematic sectional view showing a single-part type nozzle unit which is another example of a nozzle unit to which the present invention is applicable.
FIG. 3 is a graph showing the relationship between the ratio of a surface area of an inner hole of a nozzle unit to be defined by CaO-containing refractories to the entire surface area of the inner hole, and large-size alumina inclusions in obtained slabs.
FIG. 4 is a graph showing the relationship between the average amount of CaO in refractories defining a surface area of an inner hole of a nozzle unit, and large-size alumina inclusions in obtained slabs.

### BEST MODE FOR CARRYING OUT THE INVENTION

The present invention will be described in conjunction with one embodiment in which the present invention is applied to the multi-part type nozzle unit as shown in FIG. 1.

**Table 1**

| Material | | A | B | C | D |
|---|---|---|---|---|---|
| Composition (mass%) | CaO | 40 | 50 | - | - |
| | MgO | 30 | 46 | - | - |
| | Al₂O₃ | - | - | 70 | 96 |
| | C | 30 | 4 | 30 | 4 |

In the above Table 1, the respective compositions of materials applied to the segmental nozzles of the multi-part type nozzle in FIG. 1. Each of the materials A and B in Table 1 is a CaO-containing material according to the present invention, and each of the materials C and D is a comparative example containing no CaO.

Each of the materials A to D was shaped, burnt and machined to prepare sleeve-shaped refractories having a thickness of 10 mm. The sleeve-shaped refractories were inserted into the respective inner holes of the segmental nozzles, and bonded thereto with mortar to form the segmental nozzles as shown in FIG. 1. The refractories made of the material A or C were applied to the immersion nozzle, and the refractories made of the material B or D were applied to the upper nozzle, the sliding nozzle (SN) and the lower nozzle.

Table 2 shows a surface area of the inner hole of each of the segmental nozzles having the CaO-containing refractories applied thereto.

**Table 2**

| | Surface Area of Inner Hole (cm²) |
|---|---|
| Upper Nozzle | 393 |
| Sliding Nozzle | 438 |
| Lower Nozzle | 368 |
| Immersion Nozzle | 915 |

A plurality of multi-part type continuous casting nozzle units were prepared by variously combining the prepared segmental nozzles serving as the upper nozzle 2, SN 3, lower nozzle 4 and immersion nozzle in FIG. 1.

The influence of the materials used in the nozzle unit on the quality of slabs was experimentally checked to clarify effects derived from the use of the CaO-containing refractories. In the experimental tests, the casting of aluminum-killed steel was performed while changing a combination of the segmental nozzles under the casting conditions of a ladle volume: 250 ton, a TD volume: 45 ton, and a drawing speed of slabs: 1.0 to 1.3 m/min, and the effects were checked in accordance with the number per area of large-size alumina inclusions having a particle size of 50 µm or more, which were contained in obtained slabs.

**Table 3**

| | | Comparative Example | | | | | | | Inventive Example | | | | | | |
|---|---|---|---|---|---|---|---|---|---|---|---|---|---|---|---|
| | | 1 | 2 | 3 | 4 | 5 | 6 | 7 | 1 | 2 | 3 | 4 | 5 | 6 | 7 |
| Material applied to Inner Hole | Upper nozzle | D | B | D | D | D | B | D | B | D | D | B | B | B | B |
| | Sliding nozzle | D | D | B | D | D | B | B | D | B | B | B | B | D | B |
| | Lower nozzle | D | D | D | B | D | D | B | D | D | B | B | D | B | B |
| | Immersion nozzle | C | C | C | C | A | C | C | A | A | A | C | A | A | A |
| Ratio of CaO in inner hole surface Area (%)*1 | | 0 | 19 | 21 | 17 | 43 | 39 | 38 | 62 | 64 | 61 | 57 | 83 | 79 | 100 |
| Number of inclusions *2 | | 100 | 90 | 87 | 92 | 75 | 80 | 82 | 15 | 13 | 16 | 22 | 6 | 7 | 3 |

| | | | | | | | | | | | | | | | |
|---|---|---|---|---|---|---|---|---|---|---|---|---|---|---|---|
| *1 The ratio of a surface area of the inner hole defined by the CaO-containing material to the entire surface area of the inner hole *2 The number of large-size alumina inclusions (Index Number on the basis that the number of large-size alumina inclusions in Comparative Example 1 is 100) | | | | | | | | | | | | | | | |

Table 3 shows the test result. In Table 3, the number of large-size alumina inclusions in each example is shown by an index number on the basis that the number of large-size alumina inclusions in slabs obtained using the multi-part type nozzle unit in Comparative Example 1 is 100. This means that the nozzle unit having a smaller index number can provide slabs having better quality or a smaller number of large-size alumina inclusions.

FIG. 3 diagrammatically shows the result in Table 3 in the form of the relationship between the ratio of a surface area of the inner hole defined by the CaO-containing material to the entire surface area of the inner hole, and the number of large-size alumina inclusions.

As seen in FIG. 3, when the ratio of a surface area of the inner hole defined by the CaO-containing refractories to the entire surface area of the inner hole of the nozzle unit is increased up to more than 50%, the number of large-size alumina inclusions is sharply reduced to improve the quality of slabs. Then, the quality of slabs is further improved as the ratio is increased, and the best quality can be obtained when the CaO-containing refractories are applied to the entire surface area of the inner hole of the nozzle unit.

Further, in the nozzle unit as shown in FIG. 1, the influence of the amount of CaO in the CaO-containing refractories on the quality of slabs was experimentally checked.

**Table 4**

| Material | | A | B | E | F | G | H | I | J | K | L |
|---|---|---|---|---|---|---|---|---|---|---|---|
| Composition (mass%) | CaO | 40 | 50 | 10 | 15 | 20 | 30 | 10 | 15 | 20 | 30 |
| | MgO | 30 | 46 | 60 | 55 | 50 | 40 | 76 | 71 | 66 | 56 |
| | C | 30 | 4 | 30 | 30 | 30 | 30 | 4 | 4 | 4 | 4 |

As an example, Table 4 shows CaO-containing refractories having compositions E to L in addition to the compositions A and B in Table 1. As with the materials in Table 1, each of these CaO-containing refractories were shaped, burnt and machined to form sleeve-shaped refractories having a thickness of 10 mm. The sleeve-shaped refractories were inserted into the respective inner holes of the segmental nozzles, and bonded thereto with mortar to form segmental nozzles for test. The refractories made of the material A, E, F, G or H were applied to the immersion nozzle 5 in FIG. 1, and the refractories made of the material B, I, J, K or L were applied to the upper nozzle 2, the SN 3, and the lower nozzle 4 in FIG. 1.

A surface area of the inner hole of each of the segmental nozzles is the same as that shown in Table 2.

In the experimental tests, the casting was performed using each of multi-part type nozzle units prepared by variously combining these segmental nozzles in the structure as shown in FIG. 1, under the same casting conditions as those described above to check the quality of slabs. The test results are shown in Table 5. The quality of slabs was evaluated in the same manner as in Table 3.

**Table 5**

| | | Comparative Example | | Inventive Example | | |
|---|---|---|---|---|---|---|
| | | 8 | 9 | 8 | 9 | 10 |
| Material applied to Inner Hole | Upper nozzle | I | J | K | L | B |
| | Sliding nozzle | I | J | K | L | B |
| | Lower nozzle | I | J | K | L | B |
| | Immersion nozzle | E | F | G | H | A |
| Number of inclusions *1 | | 80 | 65 | 20 | 14 | 3 |

| | | | | | | |
|---|---|---|---|---|---|---|
| * 1 The number of large-size alumina inclusions (Index Number on the basis that the number of large-size alumina inclusions in Comparative Example 1 is 100) | | | | | | |

The results in Table 5 are summarized in FIG. 4 in the form of the relationship between the average amount of CaO in the refractories applied to the inner hole of the nozzle unit, and the number of large-size alumina inclusions. As seen in FIG. 4, when the average amount of CaO in the refractories applied to the inner hole of the nozzle unit is increased up to 20 mass% or more, the quality of slabs is significantly improved.

### INDUSTRIAL APPLICABILITY

The present invention can significantly reduce the amount of large-size inclusions in slabs during casting of aluminum-killed steel, and can be applied to various nozzle units irrespective of nozzle type, such as multi-part type and single-part type.

## Claims

1. A method of continuous casting of aluminum-killed steel using a continuous casting nozzle unit which is arranged of a refractory material containing CaO on a face of an inner hole of the continuous casting nozzle unit,
wherein said continuous casting nozzle unit is **characterized in that**:
a ratio of a surface area of that inner hole defined by said refractory material containing CaO to the entire surface area of that inner hole is more than 50%;
and
said refractory material is a MgO-CaO-C based refractory containing CaO from 20 to 60 wt.%.

2. A method of continuous casting of aluminum-killed steel as defined by claim 1, wherein the refractory is formed to a sleeve by shaping and burning.

3. A method of continuous casting of aluminum-killed steel as defined by claim 1 or claim 2, wherein the continuous casting nozzle unit is a combined multi-part nozzle unit.

## Patentansprüche

1. Verfahren zum Stranggießen von aluminiumberuhigtem Stahl unter Verwendung einer Stranggussdüseneinheit, welche angeordnet ist aus einem CaO enthaltenden feuerfesten Material auf einer Fläche eines Innenloches der Stranggussdüseneinheit,
wobei die Stranggussdüseneinheit **dadurch gekennzeichnet ist, dass**:
ein Verhältnis der Oberfläche dieses Innenlochs, die durch besagtes CaO enthaltendes feuerfestes Material definiert ist, zu der gesamten Oberfläche des Innenloches größer als 50% ist;
und
besagtes feuerfestes Material ein feuerfestes Material auf Basis von MgO-CaO-C ist, das von 20 bis 60 Gew.-% CaO enthält.

2. Verfahren zum Stranggießen von aluminiumberuhigtem Stahl nach Anspruch 1, wobei das feuerfeste Material durch Ausformen zu einer Hülse und Brennen geformt wird.

3. Verfahren zum Stranggießen von aluminiumberuhigtem Stahl nach Anspruch 1 oder Anspruch 2, wobei die Stranggussdüseneinheit eine kombinierte mehrteilige Düseneinheit ist.

## Revendications

1. Procédé de coulée continue d'acier calmé à l'aluminium utilisant une unité de type busette de coulée continue qui est arrangée d'un matériau réfractaire contenant du CaO sur une surface d'un trou intérieur de l'unité de type busette de coulée continue,
dans lequel ladite unité de type busette de coulée continue est **caractérisée en ce que**:
un rapport d'une surface de ce trou intérieur défini par ledit matériau réfractaire contenant du CaO à toute la surface de ce trou intérieur est supérieur à 50 % ;
et
ledit matériau réfractaire est un produit réfractaire à base de MgO-CaO-C contenant du CaO de 10 à 60 % en poids.

2. Procédé de coulée continue d'acier calmé à l'aluminium selon la revendication 1, dans lequel le produit réfractaire est formé en un manchon par formage et par cuisson.

3. Procédé de coulée continue d'acier calmé à l'aluminium selon la revendication 1 ou la revendication 2, dans lequel l'unité de type busette de coulée continue est une unité de type busette constituée de plusieurs pièces combinées.
